

March 6, 1934.

E. B. A. ZWOYER ET AL

1,950,017

METHOD OF CARBONIZING COAL BRIQUETTES

Filed Aug. 11, 1931

2 Sheets-Sheet 1



WITNESS

G. V. Rasmussen

INVENTORS  
ELLSWORTH B. A. ZWOYER  
ALBERT L. STILLMAN  
BY *Prinsen Schreuk*  
ATTORNEYS

March 6, 1934.

E. B. A. ZWOYER ET AL

1,950,017

METHOD OF CARBONIZING COAL BRIQUETTES

Filed Aug. 11, 1931

2 Sheets-Sheet 2



WITNESS

*G. V. Rasmussen*

BY

INVENTORS  
ELLSWORTH B. A. ZWOYER  
ALBERT L. STILLMAN

*Briesen Schreick*  
ATTORNEYS

## UNITED STATES PATENT OFFICE

1,950,017

METHOD OF CARBONIZING COAL  
BRIQUETTES

Ellsworth B. A. Zwoyer, Perth Amboy, and Albert L. Stillman, Plainfield, N. J., assignors to The General Fuel Briquette Corporation, New York, N. Y., a corporation of New York

Application August 11, 1931, Serial No. 556,378

7 Claims. (Cl. 202—22)

This invention relates to a method for producing smokeless fuel briquettes possessing sufficient rigidity of structure, not only during the several stages of treatment, but to withstand handling, transportation and maintain their form after ignition and while being consumed.

The type of briquettes with which the process is more particularly concerned involves the use of finely ground anthracite and a binder of coal tar pitch or sulphite pitch and molasses. The method of mixing proportioning, handling and briquetting this type of material is well known, but the briquettes as delivered by the briquetting press do not possess the necessary strength and rigidity for ordinary use nor are they smokeless. Heretofore efforts have been made to render such briquettes smokeless by exposing them to elevated temperatures, but the fluidity of the binders during the heat treatment, the movement of the briquettes in their heat softened condition upon each other, and similar conditions interferred with the successful commercial use of such process on any substantial scale. It is one of the objects of the present invention to supply a method of treatment which will be economical throughout and in which the briquettes will be subjected to a series of treatments each appropriate for the then particular condition of the briquettes.

The invention is illustrated in the drawings in which Fig. 1 illustrates a longitudinal section through the apparatus and Fig. 2 is a plan view of the apparatus shown in Fig. 1.

The temperature figures applied to these figures of the drawings are representative of conditions prevailing in one method of practicing the invention. Fig. 3 is a diagrammatic elevational view looking at the briquette conveyor 10 from the left side of Figs. 1 and 2. Fig. 4 is a similar view of a coal fines conveyor 15 viewed from the right side of Figs. 1 and 2, and Fig. 5 is a similar view illustrating the operations of the coal fines conveyor 22 viewed from the right side of Figs. 1 and 2.

In connection with these drawings it is to be presupposed that briquettes composed of about 90-94% anthracite particles and 6-10% binder constituted of coal tar and bunker C fuel oil or other suitable binding material such for example as sulphite pitch and molasses and shaped and compressed in a press such as that shown in United States Patent No. 1,627,222, are being delivered with machine like regularity to a drag chain conveyor 1. The briquettes are conveyed by this conveyor from the press to the pre-

heater chamber 2 and reach the preheater, while still retaining a temperature of approximately 150° F., remaining from the press temperature. The bottom of the conveyor trough consists of a gate extending over the entire width of the chain grate 3 in the preheating chamber 2. The design of the gate is such that it may be adjusted to any angle necessary to cause the briquettes to be deposited upon the chain grate 3 as a quiescent single layer in which the individual briquettes are substantially out of pressure contact with one another.

The chain grate 3 is endless and acts as a conveyor on which the uncarbonized briquettes are distributed in a single layer so that each may receive like treatment. The use of a standard make of roller chain 4 acting as a roller bearing, interposed between the chain grate and the supporting track 5, represents a marked improvement over other structures heretofore suggested for performing analogous service. The speed of the chain grate is such that each individual briquette will remain in the chamber 2 for a period ranging from 2 to 5 minutes depending upon the particular kind of briquettes and the variation of temperature conditions.

For the heat treatment of the briquettes, a stoker fired furnace 6 furnishes sufficient heat of sufficient uniformity for the entire carbonizing operation to which the briquettes are subjected in their passage through the entire apparatus, shown in the drawings, from the point of introduction to the point of their discharge.

The temperature of the incoming gases passing from the furnace 6 and passing into contact with the single layer of briquettes, in the preheater chamber 2, is approximately 2000° F. This approximate temperature is readily maintainable by the employment of a thermostatic furnace control (not shown). As the temperature of the briquettes is about 150° F. it is apparent that, as they enter the preheater 2, they will at once be exposed to the greatest difference in temperature and the highest temperature of the entire process. The result of this treatment is to quickly surface harden the briquettes uniformly over their entire surface to the end that they may be successfully passed through the next succeeding operation notwithstanding that the inner portions of the briquettes are still in a soft condition. This effect is most effectively accomplished by individualizing the briquettes on the chain grate for if they were in pressure contact with one another or rested one upon the other as they do on the cross conveyor 1, the heat would

not envelop the briquettes uniformly and they would be soft and misshapen at their points of compressive contact.

The temperature of the briquettes leaving the preheater 2 is approximately 950° F. while the temperature of the furnace gases leaving the preheater 2 is about 1200° to 1400° F. say 1300° F. for example, at the inlet end of the rotary carbonizer 7. The rotary carbonizer 7 may be a 10 tube approximately four feet in diameter arranged to be slowly revolved by mechanism (not shown) at a rate of about  $\frac{1}{4}$  R. P. M. In this rotary drum 7 the briquettes are rolled on each other that is, subjected in a mass to a slow 15 tumbling action, being in this way uniformly exposed to the high temperature furnace gases, until at the discharge end of the rotary drum 7 the carbonizing gases are approximately 800° F. while the temperature of the briquettes is about 20 700°. The rotary drum 7 is inclined so that the rotation of the drum causes the briquettes to travel lengthwise thereof while being gently agitated together in a rotary motion and the inclination is such that the briquettes are maintained 25 in the drum for about 15 minutes, or sufficient time to absorb the necessary heat from the furnace gases. The degree of inclination of the drum 7 can be varied to lengthen or shorten the time for the briquettes to pass through the carbonizer drum 7 according to the particular nature 30 and constitution of the briquettes. In any event care is taken at the elevated end of the drum 7 that a tight fit is provided, with the end of the preheater 2, to prevent leakage of the furnace gases and the entry of oxidizing air and temperature loss at this point. An inclined wall 8 provides a smooth, connecting guideway for the briquettes between the time they leave the chain 35 grate 3 and their entry into the drum 7.

If desired the preheater may be wider than shown in the drawing and a plurality of drums 40 may be used.

The operative rotating speed of the drum 7 is made extremely low in order to eliminate the 45 abrasive action on the briquettes, otherwise occurring in this part of the apparatus. If in connection with the particular type of briquettes, too much abrasion should manifest itself, the speed of rotation is reduced and the inclination 50 increased.

After the briquettes have passed through the drum 7 they have been almost completely carbonized and therefore rendered smokeless and by reason of the antecedent series of steps their 55 shape has been preserved and their strength greatly increased. In order, however, to store the briquettes safely it is important that their temperature should be reduced to approximately 150° F. throughout 100% of the entire mass. In other 60 words a cooling system must be provided which will reliably reduce the temperature to the stated point. Without such temperature reduction at any point, the briquettes otherwise, when stored, are likely to catch afire. Quenching with water, 65 while very effective as a temperature reducer to below the critical point, is manifestly undesirable for many reasons. Atmospheric or forced air cooling are expensive in operation and uncertain. To meet the necessary conditions, the procedure 70 now to be described was devised and found to be 100% effective, inexpensive and profitable. Speaking generally, the hot carbonized briquettes leaving the carbonizing drum 7 are first brought into intimate uniform contact with coal fines, from 75 their place of storage, on their way to the mixer

from which the briquetting press draws its supply. Such coal fines are naturally moist depending somewhat upon humidity, precipitation, length of time of storage, etc. At any rate they can be depended upon to have a moisture content of at least 15%. These moist coal fines are fed into the conveyor 10 by the conveyor 9 from an outside source of supply. The conveyor 10 passes below the discharge end of the carbonizing drum 7 and there receives the hot briquettes as they are discharged from the drum 7. The conveyor 10 is in the form of a gravity discharge bucket elevator, which retains the briquettes and the coal fines, which have been deposited upon the briquettes from the conveyor 9, until they reach the chute aperture 11 where they are dumped indiscriminately into said chute 11 and thence into the elevated end of the cooling unit 12. The nature and action of the conveyors 9 and 10 are of standard and well known type. One available variety is 80 illustrated in Fig. 3 where the chains 10a carry buckets 10b, which, moving over plate 10c, pick up the briquettes and subsequently the coal fines deposited on said plate by a scraper conveyor 9. The buckets 10b, on passing over the roller 10d, 85 deposit their contents on the plate 10e and also advance the mixed briquettes and fines into the chute 11. In the cooler 12 the wet coal and hot briquettes are now caused to intermingle thoroughly with each other by the rotary action of the 90 cooler unit 12. Moisture evaporated from the coal fines, by the heat of the briquettes, being carried away by the current of air passing counter current through the cooler 12 into the stack housing 13. The lower end of the cooler 12 comprises a 95 separating chamber in the form of a screen 14, through which the dried heated fines are discharged into the gravity discharge bucket elevator 15, while the briquettes substantially free from the screened fines, and now having a uniform 100 temperature of approximately 130° F., slide over the spout 16 into suitable vehicles or conveyors by which they are brought to storage, or 105 shipped.

The fines discharged into the elevator 15 which, 110 as illustrated in Fig. 4, operates like the conveyor 10, comprising chains 15a carrying buckets 15b, plate 15c, and plate 15e are discharged into the chute 17, which leads to the elevated end of a rotary conditioning unit 18, through which in the 115 opposite direction pass the furnace gases, from the furnace 6 after they have done their work in the preheater 2 and in the carbonizer drum 7, and where they still have a temperature of about 800° F. The coal fines entering unit 18, have a 120 temperature of about 130° F., will be raised to about 250° F. as they pass through unit 18, while the exhaust gases from the drum 7, entering unit 18 at about 800° F. are discharged into the stack 125 19 at approximately 300-400° F. Fans 20 and 21 130 maintain the proper draft requirements at the two stacks of the apparatus.

The binders used for briquettes have a melting point which, as in the case of pitch, can generally be set down as of the order of 175 to 200° F. 140 which means that in order to obtain a proper intermixture between the binders and coal fines heat must be supplied. In the present instance the coal fines being heated by the process to about 250° F. can be directly used in the mixer as a 145 source of heat to bring the binders into proper temperature and plasticity with respect to the coal fines with which they are to amalgamate thereby effecting considerable economy in their part of the operation. The hot coal fines dis- 150

charged from the unit 18 are therefore preferably transported by the bucket elevator 22 illustrated in Fig. 5 and comprising chains 22a, buckets 22b

plate 22c, and upper plate 22e, said plate 22e having its delivery point directly anterior to the mixer, or to a place of storage in the vicinity of the mixer, so that they can be used before they have lost their heat. The feed of coal fines into the conveyor 10 can be regulated in consonance with the amount required in the mixer to keep the briquetting press supplied with mixed material at the rate at which the press delivers briquetted product to the conveyor 1. It will be noted, that proceeding in this manner, there will be ample moist coal fines fed to the hot briquettes entering the cooler 12 to effect the necessary cooling of the briquettes in that unit. When starting operations after a shut down, or new installation, heat is started in furnace 6, coal fines are fed into the elevated end of unit 18 or conveyed there, if desired by elevators 9 and 10, unit 12 and elevator 15, the fines being in this way preheated for the mixing operation. After sufficient amounts of hot fines have been mixed with the binder to start supplying the press for continuous operation, the press begins its work, delivering its product to conveyor 1 and in a very short time the entire apparatus shown in the drawings will function automatically and normally in the manner hereinabove described.

The process hereinabove described lends itself to the production of satisfactory briquettes in which the binders may be of various kinds including such as contain asphaltic oil or asphalt coal tar and bunker C fuel oil or bunker C fuel oil alone. In fact so far as the use of a binder composed of bunker C fuel oil is concerned, the process hereinabove described is, so far as we are aware, the only known process by which satisfactory briquettes can be produced when that type of binder is employed. The initial high temperature treatment seems to cause reactions which leave an effective condition of cohesion in the briquettes even in those cases where asphaltic binders or similar binders, which ordinarily possess only an inferior binding capacity, are used. Thus the new process opens up fields of use for binder materials which have not thus far been usable with satisfactory effect in commercial practice.

The process described herein is particularly advantageous when used in connection with anthracite briquettes but may, of course, be employed in connection with material equivalent to anthracite in its behaviour in relation to and in response to the said process. When, therefore, in the claims we refer to anthracite coal, it is to be understood that we include equivalent material.

We claim:

1. The method of making coal briquettes, which comprises distributing raw compressed briquettes, composed of finely ground anthracite coal and a binder, as a single layer within a heating chamber and passing them through said heating chamber as a quiescent single layer in which the individual briquettes are substantially not in pressure contact with one another, subjecting said briquettes forthwith upon their entry into said chamber to high heat, maintaining said briquettes in said high heat region for a sufficient time to surface harden said briquettes but not long enough to result in combustion or to carbonize them throughout, then in a separate stage carbonizing the briquettes at a lower temperature appropriate

for thoroughly carbonizing such briquettes and simultaneously subjecting said briquettes in a mass to a slow tumbling action so that the

briquettes roll upon each other, and finally cooling the thus hardened and carbonized briquettes. 80

2. In a method of making coal briquettes containing particles of anthracite coal, the steps which comprise mixing the coal with a binder, molding carbonizable briquettes therefrom, subjecting such briquettes as a quiescent single layer in which the individual briquettes are substantially out of pressure contact with one another to a high heat for a short period to surface-harden them without carbonizing them throughout, withdrawing the briquettes from the zone of high heat, and thereupon in a separate stage subjecting said briquettes in a mass to a slow tumbling action so that the briquettes roll upon each other and during said stage carbonizing the briquettes at a lower temperature appropriate for thoroughly carbonizing such briquettes. 90

3. In the method of making coal briquettes containing particles of anthracite coal, the steps which comprise mixing the coal with a binder, molding carbonizable briquettes therefrom, subjecting such briquettes as a quiescent single layer in which the individual briquettes are substantially out of pressure contact with one another, to a high heat for a short period sufficient to merely surface-harden them, withdrawing the 105 briquettes from the influence of high heat, then carbonizing the briquettes throughout at a lower temperature appropriate for such carbonizing of said briquettes while gently agitating them together in a rotary motion, and subjecting the 110 thus carbonized briquettes to a cooling medium consisting of coal fines until the temperature of the carbonized briquettes is below approximately 150° F. 100

4. In the method of making coal briquettes 115 containing particles of anthracite coal, the steps which comprise mixing the coal with a binder, molding carbonizable briquettes therefrom, subjecting such briquettes as a quiescent single layer in which the individual briquettes are substantially out of pressure contact with one another, to a high heat for a short period sufficient to merely surface-harden them, withdrawing the briquettes from the influence of high heat, then carbonizing the briquettes throughout at a lower temperature 120 appropriate for such carbonizing of said briquettes while gently agitating them together in a rotary motion, bringing the thus carbonized briquettes into intimate contact with a cooling medium consisting of coal fines, having a temperature materially below the temperature of the briquettes, moving the briquettes and coal fines together in contact with each other until the coal fines have materially reduced the temperature of the briquettes, and separating the coal 125 fines and briquettes. 130

5. The method of making coal briquettes containing particles of anthracite coal, which comprises mixing the coal with a binder, molding carbonizable briquettes therefrom, arranging such 140 briquettes in a heating space as a quiescent single layer in which the individual briquettes are substantially out of pressure contact with one another bringing high temperature combustion gases into contact with the briquettes, moving the briquettes in such single layer arrangement through and in contact with said high temperature gases until they are surface-hardened, removing the briquettes from said heating space to a carbonizing 145 space, introducing gases from said heating space 150.

to said carbonizing space into contact with said briquettes to carbonize the same throughout while gently agitating them together in a rotary motion, bringing the thus carbonized briquettes into heat-exchange relation with coal fines, and separating the briquettes and coal fines.

6. In the method of making coal briquettes containing particles of anthracite coal, the steps which comprise mixing the coal with a binder, 10 molding carbonizable briquettes therefrom, subjecting such briquettes as a quiescent single layer in which the individual briquettes are substantially out of pressure contact with one another to a high heat for a short period sufficient to 80 merely surface-harden them, withdrawing the briquettes from the influence of high heat, then subjecting the briquettes while gently agitating them together in a rotary motion to a lower temperature to carbonize the same throughout, 85 bringing the thus carbonized briquettes into intimate contact with moist coal fines, having a temperature materially below the temperature of the briquettes, retaining the briquettes and coal fines in contact with each other until the coal fines have materially reduced the temperature of the briquettes, separating the coal fines and briquettes, and sweeping a countercurrent of air over said coal fines to remove the moisture evaporated from said fines.

15 20 25 30 35 40 45 50 55 60 65 70 75

7. In a method of making coal briquettes containing particles of anthracite coal, the steps which comprise mixing the coal with a binder,

molding carbonizable briquettes therefrom, subjecting such briquettes as a quiescent single layer in which the individual briquettes are substantially out of pressure contact with one another to a high heat for a short period sufficient to 80 merely surface-harden them, withdrawing the briquettes from the influence of high heat, then subjecting the briquettes while gently agitating them together in a rotary motion to a lower temperature to carbonize the same throughout, 85 bringing the thus carbonized briquettes into intimate contact with moist coal fines, having a temperature materially below the temperature of the briquettes, retaining the briquettes and coal fines in contact with each other until the coal fines have materially reduced the temperature of the briquettes, separating the coal fines and briquettes, and sweeping a countercurrent of air over said coal fines to remove the moisture evaporated from said fines.

95

96

97

98

ELLSWORTH B. A. ZWOYER.  
ALBERT L. STILLMAN.

100

105

110

115

120

125

130

135

140

145

150